



US006132943A

**United States Patent** [19]**Younathan et al.****Patent Number:** **6,132,943****Date of Patent:** **Oct. 17, 2000**[54] **COLOR PHOTOGRAPHIC ELEMENTS  
CONTAINING YELLOW-COLORED  
MAGENTA DYE-FORMING MASKING  
COUPLERS**[75] Inventors: **Janet N. Younathan**, Fairport, N.Y.;  
**Michael W. Crawley**, Watford, United  
Kingdom; **Krishnan Chari**, Fairport,  
N.Y.[73] Assignee: **Eastman Kodak Company**, Rochester,  
N.Y.[21] Appl. No.: **09/418,392**[22] Filed: **Oct. 14, 1999**[51] **Int. Cl.<sup>7</sup>** ..... **G03C 1/46**[52] **U.S. Cl.** ..... **430/504**; 430/555; 430/359;  
430/559; 430/561; 430/562; 430/558[58] **Field of Search** ..... 430/555, 504,  
430/359, 559, 561, 562, 558, 563[56] **References Cited**

## U.S. PATENT DOCUMENTS

|           |         |                              |
|-----------|---------|------------------------------|
| 1,055,155 | 3/1913  | Fischer .                    |
| 2,376,679 | 5/1945  | Frohlich et al. .            |
| 2,428,054 | 9/1947  | Vittum et al. .              |
| 2,808,329 | 10/1957 | Whitmore .                   |
| 2,852,370 | 9/1958  | Whitmore .                   |
| 3,227,550 | 1/1966  | Whitmore et al. .            |
| 4,004,929 | 1/1977  | Orvis .                      |
| 4,070,191 | 1/1978  | Imamura et al. .             |
| 4,163,670 | 8/1979  | Shiba et al. .               |
| 5,219,719 | 6/1993  | Kida .                       |
| 5,241,058 | 8/1993  | Renner et al. .              |
| 5,466,568 | 11/1995 | Kapp et al. .                |
| 5,492,799 | 2/1996  | Kapp et al. .                |
| 5,622,818 | 4/1997  | Kapp et al. .                |
| 5,853,971 | 1/2000  | Bell et al. ..... 430/555    |
| 6,010,839 | 1/2000  | Crawley et al. ..... 430/558 |

## FOREIGN PATENT DOCUMENTS

7120901 5/1995 Japan .

*Primary Examiner*—Geraldine Letscher  
*Attorney, Agent, or Firm*—Andrew J. Anderson[57] **ABSTRACT**

A multilayer silver halide color photographic element is disclosed comprising a support bearing a light-sensitive silver halide emulsion layer and a non-diffusible yellow-colored magenta dye-forming masking coupler of the following formula



wherein COUP is a magenta dye-forming coupler having the azo group attached to its coupling position; q is an integer of from 0 to 3, and each R' independently represents a substituent group or two R' groups together complete a ring of from 5-7 atoms, which ring may include 1 or more heteroatoms selected from O, N and S; m is 1 or 2, and DG represents a substituent of the formula



where each L<sup>1</sup> represents a divalent linking group, preferably  $-\text{O}(\text{CH}_2)_y-$ ,  $-\text{NHCO}(\text{CH}_2)_y-$ , or  $-\text{NRCO}(\text{CH}_2)_y-$ , where R represents an alkyl or aryl group and y represents an integer from 1 to 4; each k is either 0 or 1; each L<sup>2</sup> represents  $-\text{NHSO}_2-$ ,  $-\text{NHCO}-$ ,  $-\text{SO}_2\text{NH}-$ , or  $-\text{CONH}-$ , preferably at least one L<sup>2</sup> group being  $-\text{NHSO}_2-$  or  $-\text{SO}_2\text{NH}-$ , more preferably  $-\text{NHSO}_2-$ ; each Z represents  $-\text{SO}_3\text{M}$  or  $-\text{PO}_3\text{M}$ , where M represents H or a counter ion such as Na, K, Li, or NH<sub>4</sub>; and each n represents an integer of from 1 to 5; with the provisos that each DG substituent group, when present, is located in the 4- or 6-position meta to the 2-hydroxyl substituent on the arylazo group, and that when at least one L<sup>1</sup> or L<sup>2</sup> group comprises an  $-\text{NHSO}_2-$  or  $-\text{SO}_2\text{NH}-$  group then the total number of Z group substituents on the coupler is at least 2, and when no L<sup>1</sup> or L<sup>2</sup> group comprises an  $-\text{NHSO}_2-$  or  $-\text{SO}_2\text{NH}-$  group then the total number of Z group substituents on the coupler is at least 3, and if k is 0 for a DG substituent group then the L<sup>2</sup> group for that DG substituent is either  $-\text{NHSO}_2-$  or  $-\text{NHCO}-$ .

**27 Claims, No Drawings**

**COLOR PHOTOGRAPHIC ELEMENTS  
CONTAINING YELLOW-COLORED  
MAGENTA DYE-FORMING MASKING  
COUPLERS**

**FIELD OF THE INVENTION**

This invention relates to color photographic elements containing particular magenta dye-forming masking couplers.

**BACKGROUND OF THE INVENTION**

Most silver halide color photographic elements form multicolor images in the element by subtractive color mixing. This involves the formation of yellow, magenta and cyan dye images by color development of imagewise exposed blue, green and red sensitive silver halide emulsion layers. Ideally, the subtractive dyes so formed should absorb radiation only in the region of the spectrum which is the complement of the region of exposure. Unfortunately, all dyes have some unwanted side absorptions. To correct for these unwanted side absorptions it is common practice for color negative photographic elements to employ one or more colored masking couplers. These couplers have a color which is similar to the unwanted side absorption of one of the dyes formed from one of the image couplers. The color of the masking coupler is destroyed in the areas of the image where the dye with unwanted side absorptions is formed. The way in which colored masking couplers are employed to correct for the unwanted side absorption is described in more detail in J. Phot. Soc. Am. 13, 94(1947), J. Opt. Soc. Am. 40, 166(1950) and J. Am. Chem. Soc. 72, 1533(1950).

A preferred class of colored masking couplers are the 4-phenylazo-5-pyrazolones which correct for the unwanted yellow side absorption of magenta dye-forming couplers. Such couplers have found widespread use in color photographic elements. It is known that certain substituents on the 4-arylazo group are useful. Included, e.g., are alkoxy, hydroxy, and carbonamido groups, usually in the para position to the azo function. It has been customary to include such substituents as will permit or indeed improve the propensity of the decoupled arylazo residue to be washed out of the film during processing. The masking coupler itself, however, typically includes a hydrophobic ballast group to confer non-diffusibility to the coupler, and such masking couplers are typically dispersed in aqueous coating solutions with high boiling permanent organic solvents, known in the art as coupler solvents, using conventional homogenization dispersion techniques. Coupler solvents are generally required to provide adequate coupler activity, but excess solvent can result in increased material loads resulting in increased photographic layer thickness, which may negatively impact the optical properties of the film. High solvent levels may also raise ecological concerns.

U.S. Pat. No. 5,622,818 discloses 4-phenylazo-5-pyrazolone masking compounds in which the phenylazo coupling-off group is 2-hydroxy-5-substituted. These couplers are advantageous with respect to other substitution patterns on conventional solvent dispersed masking couplers as they are easier to synthesize than masking compounds where the coupling-off group is 2-hydroxy-4-substituted. The ease of synthesis arises from the substitution pattern (on 2 and 5 positions) of the arylazo ring, because this pattern reduces the possibility of isomer formation during the preparation of the corresponding nitrophenol, a precursor to the phenylazo coupling-off group.

Alternatives to dispersing hydrophobic photographic couplers with high boiling solvents have been suggested. Water

soluble or dispersible "Fischer-type" incorporated couplers, e.g., may be used in photographic elements, such as those described in U.S. Pat. No. 1,055,155, issued Mar. 4, 1913, and particularly non-diffusible Fischer-type couplers containing branched hydrocarbon chains, e.g., those referred to in the references cited in Frohlich et al, U.S. Pat. No. 2,376,679, issued May 22, 1945, Column 2, lines 50-60. Fischer-type couplers form self-assembled micellar aggregates in water, and may be directly incorporated in film or photographic systems without the need for a dispersion making step. Such micelle forming couplers typically comprise strong acid moieties, however, and typically interact with gelatin in coating formulations to cause high viscosities and coating defects. Additionally, such couplers may not provide desired levels of activity in comparison to conventional solvent dispersions.

Copending U.S. Ser. No. 09/105,507 filed Jun. 26, 1998 (and corresponding UK Application No. 9914155.8) describe a multilayer silver halide color photographic element comprising a support bearing a light-sensitive silver halide emulsion layer and a non-diffusible yellow-colored magenta dye-forming masking coupler of the formula



wherein COUP is a magenta dye-forming coupler having the azo group attached to its coupling position; ARYL, represents an aromatic group, including optionally further substituted phenyl, naphthyl or heteroaryl groups; m represents an integer of from 1 to 4; each L<sup>1</sup> represents a divalent linking group, preferably —O(CH<sub>2</sub>)<sub>y</sub>—, —NHCO(CH<sub>2</sub>)<sub>y</sub>—, or —NRCO(CH<sub>2</sub>)<sub>y</sub>—, where R represents an alkyl or aryl group and y represents an integer from 1 to 4; each k is either 0 or 1; each L<sup>2</sup> represents —NHSO<sub>2</sub>—, —NHCO—, —SO<sub>2</sub>NH—, or —CONH—, preferably at least one L<sup>2</sup> group being —NHSO<sub>2</sub>— or —SO<sub>2</sub>NH—, more preferably —NHSO<sub>2</sub>—; each Z represents —SO<sub>3</sub>M or —PO<sub>3</sub>M, where M represents H or a counter ion such as Na, K, Li, or NH<sub>4</sub>; and n represents an integer of from 1 to 5, with the provisos that when at least one L<sup>1</sup> or L<sup>2</sup> group comprises an —NHSO<sub>2</sub>— or —SO<sub>2</sub>NH— group then the total number of Z group substituents on the coupler is at least 2, and when no L<sup>1</sup> or L<sup>2</sup> group comprises an —NHSO<sub>2</sub>— or —SO<sub>2</sub>NH— group then the total number of Z group substituents on the coupler is at least 3, and if k is 0 for a substituent on the ARYL group then the L<sup>2</sup> group for that substituent is either —NHSO<sub>2</sub>— or —NHCO—. Masking couplers comprising the requisite number and types of L<sup>1</sup>, L<sup>2</sup> and Z groups have been found to form self-assembled micellar aggregates in water, and accordingly may be directly incorporated in aqueous solutions without the need for a dispersion making step. The specific couplers disclosed in U.S. Ser. No. 09/105,507, however, have been found to 45 demonstrate undesired fog levels in fresh photosensitive layer coatings.

It would be desirable to provide masking couplers which may be directly incorporated into an aqueous coating solution without the need for a dispersion-making step and associated organic solvents, while still providing good activity levels without the generation of undesirable levels of fog. Such couplers would enable improved photographic ele-

ments obtained by simplified photographic element manufacturing techniques and also desirably enable elements to be prepared with thinner imaging layers due to the absence of solvents otherwise needed for dispersing the couplers.

#### SUMMARY OF THE INVENTION

The present invention provides a multilayer silver halide color photographic element comprising a support bearing a light-sensitive silver halide emulsion layer and a non-diffusible yellow-colored magenta dye-forming masking coupler of the following formula



wherein

COUP is a magenta dye-forming coupler having the azo group attached to its coupling position;  
q is an integer of from 0 to 3, and each R' independently represents a substituent group or two R' groups together complete a ring of from 5-7 atoms, which ring may include 1 or more heteroatoms selected from O, N and S;  
m is 1 or 2, and DG represents a substituent of the formula



where

each L<sup>1</sup> represents a divalent linking group, preferably —O(CH<sub>2</sub>)<sub>y</sub>—, —NHCO(CH<sub>2</sub>)<sub>y</sub>—, or —NRCO(CH<sub>2</sub>)<sub>y</sub>—, where R represents an alkyl or aryl group and y represents an integer from 1 to 4;

each k is either 0 or 1;

each L<sup>2</sup> represents —NHSO<sub>2</sub>—, —NHCO—, —SO<sub>2</sub>NH—, or —CONH—, preferably at least one L<sup>2</sup> group being —NHSO<sub>2</sub>— or —SO<sub>2</sub>NH—, more preferably —NHSO<sub>2</sub>—;

each Z represents —SO<sub>3</sub>M or —PO<sub>3</sub>M, where M represents H or a counter ion such as Na, K, Li, or NH<sub>4</sub>; and each n represents an integer of from 1 to 5,

with the provisos that each DG substituent group, when present, is located in the 4- or 6-position meta to the 2-hydroxyl substituent on the arylazo group, and that when at least one L<sup>1</sup> or L<sup>2</sup> group comprises an —NHSO<sub>2</sub>— or —SO<sub>2</sub>NH— group then the total number of Z group substituents on the coupler is at least 2, and when no L<sup>1</sup> or L<sup>2</sup> group comprises an —NHSO<sub>2</sub>— or —SO<sub>2</sub>NH— group then the total number of Z group substituents on the coupler is at least 3, and if k is 0 for a DG substituent group then the L<sup>2</sup> group for that DG substituent is either —NHSO<sub>2</sub>— or —NHCO—.

Masking couplers comprising the requisite number and types of L<sup>1</sup>, L<sup>2</sup> and Z groups in accordance with the invention have been found to form self-assembled micellar aggregates in water, and accordingly may be directly incorporated in aqueous solutions without the need for a disper-

sion making step. The presence of a 2-hydroxyl group on the arylazo group has been found to result in substantially improved low fog levels in coated photographic elements, and the positioning of the DG dispersing group substituent in the 4- and/or 6-position (i.e., meta to the hydroxyl group) on the arylazo group facilitates synthesis of the described masking couplers. Further, such couplers exhibit good activity in the reaction with oxidized developer even in the absence of permanent solvent or plasticizer. While micelle forming couplers comprising strong acid moieties may in some instances interact with gelatin in coating formulations to cause high viscosities and coating defects, the masking couplers of the invention are typically used at relatively low laydowns in comparison to the primary magenta image-forming couplers of the photographic material, thus minimizing any of such potential problems.

#### DETAILED DESCRIPTION OF THE INVENTION

In accordance with the invention, water dispersable masking couplers are described comprising substituted arylazo coupling-off groups, where such coupling-off groups comprise a 2-hydroxyl substituent group and at least one dispersing group substituent of the formula DG in a meta position relative to the hydroxyl group. Where only one dispersing group substituent is present on the aryl azo group, it may be in either the 4- or 6-position, but in accordance with preferred embodiments such group is present in the 4-position. Where two DG substituents are present, they are in the 4- and 6-position s of the arylazo group.

The masking couplers employed in accordance with the invention contain dispersing or solubilizing groups which are not found on traditional solvent-dispersed masking compounds. These groups are attached in a substituent on the arylazo coupling-off group and dictate a different synthetic method than that used to prepare the coupling-off group of traditional solvent dispersed masking compounds. For example, during synthesis of masking compounds in accordance with the invention, a basic hydrolysis reaction may be used to produce an arylsulphonic acid from a corresponding difluorosulphonylarene, as indicated in the synthesis example below. This step will not proceed successfully if the hydroxyl group and the dispersing group are positioned ortho or para to one another, a substitution pattern analogous to the 2-hydroxy-5-substitution described in U.S. Pat. No. 5,622,818, as deleterious side reactions occur under the basic reaction conditions. Thus, the disclosed synthetic advantage associated with 2-hydroxy-5-substitution in conventional solvent dispersed masking compounds as taught in U.S. Pat. No. 5,622,818 cannot be realized in preparing the masking compounds in accordance with the invention.

The masking couplers of the invention may include additional substituents R' on the arylazo coupling-off groups which do not significantly detrimentally effect the performance of the coupler. Where only one DG dispersing group is present on the arylazo group in the 4-position, a second hydroxyl group may be present on the arylazo group in the 6-position. Preferably, any additional substituents on the arylazo group have a Hammett sigma-para value of less than 0.05, preferably less than 0.0, or two such additional substituents together complete a ring of from 5-7 atoms, which ring may include 1 or more heteroatoms selected from O, N and S.

In a preferred embodiment, the colored coupler is of the formula:

pyrazolotriazole compounds of the general formulas:



5

(M-3)



and

(M-4)



wherein:

q is an integer of from 0 to 3, and each R' independently represents a substituent group with a Hammett sigma-  
para value of less than 0.05, preferably less than 0.0, or  
two R' groups together complete a ring of from 5-7  
atoms, which ring may include 1 or more heteroatoms  
selected from O, N and S.

In addition to a second hydroxyl group in the 6-position as discussed above, each R' independently may be, e.g., an alkyl group, an aryl group, an amino group, an amido group, a ureido group, an alkoxy group, a sulfonamido group, or an aryloxy group, or two R' groups may represent an alkylene group or a dioxyalkylene group. Preferably, however, q is 0. If present, any R' groups preferably represent OR, R, NHCOR, 6-OH, 6-NHSO<sub>2</sub>R, or 6-NR<sub>2</sub>, where R represents an alkyl or aryl group.

Hammett sigma-para values are a measure of the electron-donating propensity of the substituent, and are described in *Substituent Constants for Correlation Analysis in Chemistry and Biology*, C. Hansch and A. J. Leo, Wiley, New York, 1979. Preferably, the substituents individually have Hammett sigma-para values in the range of -0.10 to -0.35 and together all R' groups have Hammett sigma-para values in the range of -0.10 to -0.50.

Examples of suitable R' groups are straight or branched alkyl, such as methyl, ethyl, n-propyl, i-propyl, n-butyl, s-butyl, t-butyl, t-amyl, n-dodecyl, 1,1,3,3-tetramethylbutyl and 3-(2,4-di-t-amylphenoxy)propyl; straight or branched alkoxy, such as methoxy, ethoxy and t-butoxy; aryl, such as phenyl, 4-t-butylphenyl and 2,4,6-trimethylphenyl; aryloxy, such as phenoxy and 2-methylphenoxy; ureido, such as phenylureido and methylureido; amido, such as acetamido and pivalamido; amino, such as dimethylamino and morpholino; or two R' groups together are an alkylene group such as n-propylene, n-butylene, n-pentylene and n-hexylene.

COUP can be any magenta dye-forming coupler parent. Representative magenta dye-forming couplers comprise pyrazolone compounds of the general formulas:

(M-1)



55

(M-2)



60

R<sup>3</sup> and R<sup>4</sup> are individually selected from the group consisting of hydrogen, substituted and unsubstituted alkyl, substituted and unsubstituted phenyl, substituted and unsubstituted alkoxy, substituted and unsubstituted amino, substituted and unsubstituted anilino, substituted and unsubstituted acylamino, halogens and a group which links to a polymer, provided that the total number of carbon atoms contained in R<sup>3</sup> and R<sup>4</sup> is at least 6 if neither R<sup>3</sup> nor R<sup>4</sup> is a group which links to a polymer; and

X represents the coupling-off position.

In preferred embodiments of the invention, COUP is a 5-pyrazolone dye-forming coupler. Particularly preferred couplers are 5-pyrazolone couplers having an anilino group in the 3-position. Such couplers may be represented by the structure:



(M-6)

5

10

wherein:

Ar is as defined above; and

Y is an anilino group substituted with one or more substituents selected from the group consisting of halogen atoms, and alkyl, aryl, alkoxy, aryloxy, carbonamido, carbamoyl, sulfonamido, sulfamoyl, alkylsulfinyl, arylsulfinyl, alkylsulfonyl, arylsulfonyl, alkoxycarbonyl, aryloxycarbonyl, acyl, acyloxy, ureido, imido, carbamate, heterocyclic, cyano, trifluoromethyl, alkylthio, nitro, carboxyl and hydroxyl groups, and groups which form a link to a polymeric chain, and wherein Y contains at least 6 carbon atoms.

Particularly preferred are compounds in which Ar is of the structure:



wherein R<sub>1</sub> is selected from the group consisting of halogen atoms and cyano, alkylsulfonyl, arylsulfonyl, sulfamoyl, sulfonamido, carbamoyl, carbonamido, alkoxy, acyloxy, aryloxy, alkoxycarbonyl, aryloxycarbonyl, ureido, nitro, alkyl, and trifluoromethyl groups; and

Y is of the structure:



wherein

is from zero to 2 and each R<sub>2</sub> is in a meta or para position with respect to R<sub>3</sub>;

each R<sub>2</sub> is individually selected from the group consisting of halogen, alkyl, aryl, alkoxy, aryloxy, carbonamido, carbamoyl, sulfonamido, sulfamoyl, alkylsulfinyl, arylsulfinyl, alkylsulfonyl, arylsulfonyl, alkoxycarbonyl, aryloxycarbonyl, acyl, acyloxy, ureido, imido, carbamate, heterocyclic, cyano, trifluoromethyl, alkylthio, nitro, carboxyl and hydroxyl groups; and

R<sub>3</sub> is selected from the group consisting of hydrogen, halogen, alkyl, aryl, alkoxy, aryloxy, alkylthio, carbonamido, carbamoyl, sulfonamido, sulfamoyl, alkylsulfinyl, arylsulfinyl, alkylsulfonyl, arylsulfonyl, alkoxycarbonyl, acyloxy, acyl, cyano, nitro and trifluoromethyl groups.

The masking couplers of this invention are rendered

non-diffusible as coated in the photographic element by the presence on the coupler of a ballast group. A ballast group is a group of such size and configuration that, in combination with the remainder of the molecule, it provides the coupler with sufficient bulk to be substantially non-diffusible from the layer in which it is coated in the element. The ballast group is preferably part of COUP, as is the case with dye-image forming couplers. Alternatively, the ballast group can be on the phenylazo group, in which case the dye formed on coupling may be diffusible. Representative ballast groups include alkyl or aryl groups containing 6 to 32 carbon atoms. Other ballast groups include alkoxy, aryloxy, arylthio, alkylthio, alkoxy carbonyl, aryloxy carbonyl, carboxy, acyl, acyloxy, carbonamido, carbamoyl, alkyl carbonyl, aryl carbonyl, alkylsulfonyl, arylsulfonyl, sulfamoyl, sulfenamoyl, sulfonamido, alkylsulfinyl, arylsulfinyl, alkylphosphonyl, alkoxyphosphonyl, and arylphosphonyl of 6 to 32 carbon atoms.

As used herein, unless otherwise indicated the alkyl and aryl groups, and the alkyl and aryl portions of other substituent groups, can be unsubstituted or substituted with non-interfering substituents. Typical alkyl groups have 1 to 32 carbon atoms and typical aryl groups have 6 to 32 carbon atoms. Depending upon the position of the group, preferred alkyl groups can have 1 to 20 carbon atoms, 1 to 12 carbon atoms or 1 to 4 carbon atoms and preferred aryl groups can have 6 to 20 or 6 to 10 carbon atoms. Other groups which contain a replaceable hydrogen atom can be substituted or not, depending on the particular structure and properties desired.

Throughout this application a reference to any type of chemical "group" includes both the unsubstituted and substituted forms of the group described. Generally, unless otherwise specifically stated, substituent groups usable on couplers herein include any groups, whether substituted or unsubstituted, which do not destroy properties necessary for their use as masking couplers. Examples of substituents on any of the mentioned groups can include known substituents, such as: halogen, for example, chloro, fluoro, bromo, iodo; alkoxy, particularly those with 1 to 6 carbon atoms (for example, methoxy, ethoxy); substituted or unsubstituted alkyl, particularly lower alkyl (for example, methyl, trifluoromethyl); alkenyl or thioalkyl (for example, methylthio or ethylthio), particularly either of those with 1 to 6 carbon atoms; substituted and unsubstituted aryl, particularly those having from 6 to 20 carbon atoms (for example, phenyl); and substituted or unsubstituted heteroaryl, particularly those having a 5 or 6-membered ring containing 1 to 3 heteroatoms selected from N, O, or S (for example, pyridyl, thienyl, furyl, pyrrolyl). Alkyl substituents may specifically include "lower alkyl", that is having from 1 to 6 carbon atoms, for example, methyl, ethyl, butyl, hexyl. Further, with regard to any alkyl group, alkylene group or alkenyl group, it will be understood that these can be branched or unbranched and include ring structures.

Table I, below, depicts as COUP-1 through COUP-21 examples of preferred pyrazolone coupler parents to whose coupling position (represented by a single bond in the 4-position of the pyrazolone ring) an arylazo group can be joined. COUP-22 through COUP-24 represent additional magenta dye forming coupler parents which may be used in accordance with the invention, wherein the coupling position is indicated by X.

Table II, below, depicts as AZ-1 through AZ-11 arylazo groups which may be used in accordance with the invention.

Table III, below, depicts as I-1 through I-9 representative colored masking couplers in accordance with the invention.

TABLE I



TABLE I-continued

|         |  |
|---------|--|
| COUP-6  |  |
| COUP-7  |  |
| COUP-8  |  |
| COUP-9  |  |
| COUP-10 |  |

TABLE I-continued

COUP-11



COUP-12



COUP-13



COUP-14



COUP-15



TABLE I-continued

| COUP-16 |  |
|---------|--|
| COUP-17 |  |
| COUP-18 |  |
| COUP-19 |  |
| COUP-20 |  |

TABLE I-continued



TABLE II

TABLE II-continued



TABLE II-continued

AZ-3



AZ-4



AZ-5



AZ-6



AZ-7



TABLE II-continued

AZ-8

10  
15

AZ-9

20  
25

30

AZ-10

35  
40

45

AZ-11

50  
55

60

65

TABLE III



TABLE III-continued

I-4



I-5



I-6



TABLE III-continued

I-7



I-8



TABLE III-continued



The masking couplers of this invention can be prepared by synthetic techniques well known to those skilled in the chemical art. An illustrative synthesis is shown in the Examples below.

The masking couplers of the invention are typically coated in the element at coverages of less than  $0.4 \text{ mmol/m}^2$ , preferably at a coverage of from  $0.1 \text{ mmol/m}^2$  to  $0.3 \text{ mmol/m}^2$ , and more preferably at a coverage of from  $0.18$  to  $0.24 \text{ mmol/m}^2$ . Primary magenta dye image-forming couplers, in contrast, are typically present in photographic elements at coverages of  $0.4 \text{ mmol/m}^2$  and above, most typically at a coverage of from  $0.4 \text{ mmol/m}^2$  to  $0.9 \text{ mmol/m}^2$ .

The color photographic element of this invention comprises, in addition to the magenta coupler-containing layer, various other layers typically included in color photographic elements. Multicolor color photographic elements typically contain image dye-forming units sensitive to each of the three primary regions of the visible spectrum. Each unit can comprise a single emulsion layer or multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

A typical multicolor photographic element comprises a support bearing a cyan dye image-forming unit comprised of at least one red-sensitive silver halide emulsion layer having associated therewith at least one cyan dye-forming coupler, a magenta dye image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler. The element can contain additional layers, such as filter layers, interlayers, overcoat layers, and subbing layers.

The masking couplers of the invention may be used in a photographic element in combination with any conventional primary magenta dye-forming couplers, such as those of the above formulas M-1 through M-6, wherein X represents H or a coupling-off group. Coupling-off groups are well known

25 to those skilled in the photographic art. Generally, such groups determine the equivalency of the coupler and modify the reactivity of the coupler. Coupling-off groups can also advantageously affect the layer in which the coupler is  
30 coated or other layers in the photographic material by performing, after release from the coupler, such functions as development inhibition, bleach acceleration, color correction, and development acceleration. Representative coupling-off groups include halogens (for example, chloro),  
35 alkoxy, aryloxy, alkylthio, arylthio, acyloxy, sulfonamido, carbonamido, arylazo, nitrogen-containing heterocyclic groups such as pyrazolyl and imidazoyl, and imido groups such as succinimido and hydantoinyl groups. Except for the halogens, these groups may be substituted if desired.  
40 Coupling-off groups are described in further detail in: U.S. Pat. Nos. 2,355,169; 3,227,551; 3,432,521; 3,476,563; 3,617,291; 3,880,661; 4,052,212 and 4,134,766, and in British Patent References Nos. 1,466,728; 1,531,927; 1,533,039; 2,006,755A and 2,017,704A, the disclosures of which  
45 are incorporated herein by reference.

Photographic elements of this invention can have the structures and components shown on Research Disclosure, February 1995, Item 37038, pages 79-114. Research Disclosure is published by Kenneth Mason Publications, Ltd.,  
50 Dudley Annex, 12a North Street, Emsworth, Hampshire P010 7DQ, ENGLAND. Photographic elements of the present invention can be imagewise exposed and processed using known techniques and compositions, including those described in the Research Disclosure Item 37038 cited above.  
55

If desired, the photographic element can be used in conjunction with an applied magnetic layer as described in *Research Disclosure*, November 1992, Item 34390.

A typical color negative film construction useful in the 60 practice of the invention is illustrated by the following:

| Element SCN-1 |     |                           |
|---------------|-----|---------------------------|
| 65            | SOC | Surface Overcoat          |
|               | BU  | Blue Recording Layer Unit |

-continued

| Element SCN-1 |                            |
|---------------|----------------------------|
| IL1           | First Interlayer           |
| GU            | Green Recording Layer Unit |
| IL2           | Second Interlayer          |
| RU            | Red Recording Layer Unit   |
| S             | Support                    |
| AHU           | Antihalation Layer Unit    |
| SOC           | Surface Overcoat           |

The support S can be either reflective or transparent, the latter being usually preferred. When reflective, the support is white and can take the form of any conventional support currently employed in color print elements. When the support is transparent, it can be colorless or tinted and can take the form of any conventional support currently employed in color negative elements—e.g., a colorless or tinted transparent film support. Details of support construction are well understood in the art. Transparent and reflective support constructions, including subbing layers to enhance adhesion, are disclosed in *Research Disclosure*, Item 38957, cited above, XV. Supports.

Each of blue, green and red recording layer units BU, GU and RU are formed of one or more hydrophilic colloid layers and contain at least one radiation-sensitive silver halide emulsion and coupler, including at least one dye image-forming coupler. In the simplest contemplated construction each of the layer units consists of a single hydrophilic colloid layer containing emulsion and coupler. When coupler present in a layer unit is coated in a hydrophilic colloid layer other than an emulsion containing layer, the coupler containing hydrophilic colloid layer is positioned to receive oxidized color developing agent from the emulsion during development. Usually the coupler containing layer is the next adjacent hydrophilic colloid layer to the emulsion containing layer.

The emulsion in BU is capable of forming a latent image when exposed to blue light. When the emulsion contains high bromide silver halide grains and particularly when minor (0.5 to 20, preferably 1 to 10, mol percent, based on silver) amounts of iodide are also present in the radiation-sensitive grains, the native sensitivity of the grains can be relied upon for absorption of blue light. Preferably, however, the emulsion is spectrally sensitized with one or more blue spectral sensitizing dyes. The emulsions in GU and RU are spectrally sensitized with green and red spectral sensitizing dyes, respectively, in all instances, since silver halide emulsions have no native sensitivity to green and/or red (minus blue) light.

Any convenient selection from among conventional radiation-sensitive silver halide emulsions can be incorporated within the layer units. Most commonly high bromide emulsions containing a minor amount of iodide are employed. To realize higher rates of processing high chloride emulsions can be employed. Radiation-sensitive silver chloride, silver bromide, silver iodo-bromide, silver iodo-chloride, silver chlorobromide, silver bromochloride, silver iodo-chlorobromide and silver iodo-bromochloride grains are all contemplated. The grains can be either regular or irregular (e.g., tabular). Tabular grain emulsions, those in which tabular grains account for at least 50 (preferably at least 70 and optimally at least 90) percent of total grain projected area are particularly advantageous for increasing speed in relation to granularity. To be considered tabular a grain requires two major parallel faces with a ratio of its equivalent circular diameter (ECD) to its thickness of at

least 2. Specifically preferred tabular grain emulsions are those having a tabular grain average aspect ratio of at least 5 and, optimally, greater than 8. Preferred mean tabular grain thicknesses are less than 0.3  $\mu\text{m}$  (most preferably less than 0.2  $\mu\text{m}$ ). Ultrathin tabular grain emulsions, those with mean tabular grain thicknesses of less than 0.07  $\mu\text{m}$ , are specifically preferred. The grains preferably form surface latent images so that they produce negative images when processed in a surface developer.

Illustrations of conventional radiation-sensitive silver halide emulsions are provided by *Research Disclosure*, Item 38957, cited above, I. Emulsion grains and their preparation. Chemical sensitization of the emulsions, which can take any conventional form, is illustrated in section IV. Chemical sensitization. Spectral sensitization and sensitizing dyes, which can take any conventional form, are illustrated by section V. Spectral sensitization and desensitization. The emulsion layers also typically include one or more antifogants or stabilizers, which can take any conventional form, as illustrated by section VII. Antifogants and stabilizers.

BU contains at least one yellow dye image-forming coupler, GU contains at least one magenta dye image-forming coupler, and RU contains at least one cyan dye image-forming coupler. Any convenient combination of conventional dye image-forming couplers can be employed. Conventional dye image-forming couplers are illustrated by *Research Disclosure*, Item 38957, cited above, X. Dye image formers and modifiers, B. Image-dye-forming couplers.

As in conventional color negative film constructions, RU, GU and BU can contain other colored masking couplers in addition to those in accordance with the invention.

Development inhibitor releasing compound is typically incorporated in at least one and, preferably, each of the layer units. DIRs are commonly employed to improve image sharpness and to tailor dye image characteristic curve shapes. The DIRs contemplated for incorporation in the color negative elements of the invention can release development inhibitor moieties directly or through intermediate linking or timing groups. The DIRs are contemplated to include those that employ anchimeric releasing mechanisms. Illustrations of development inhibitor releasing couplers and other compounds useful in the color negative elements of this invention are provided by *Research Disclosure*, Item 38957, cited above, X. Dye image formers and modifiers, C. Image dye modifiers, particularly paragraphs (4) to (11).

The following examples further illustrate this invention.

## SYNTHESIS EXAMPLE

Coupler I-1 was prepared according to the following synthetic scheme:

Preparation of N-[4-(3,5-bis-fluorosulphonylphenyl)sulphamoyl]-2-hydroxyphenyl]acetanilide



**31**

-continued

**32**

Preparation of Coupler I-1



N-(4-acetamido-2-hydroxyphenyl)acetamide (5.0 g, 30.1 mmol) was dissolved in dry tetrahydrofuran (50 ml) and pyridine (50 ml). A solution of 3,5-bis-fluorosulphonylbenzenesulphonamide (10.3 g, 30.2 mmol) in dry tetrahydrofuran (50 ml) was added portionwise with stirring to give a dark red solution. After stirring for 45 min, a TLC (1:1 ethyl acetate:petrol) showed the absence of the amine function (negative amine spray test), one major product spot, and several minor impurities. The reaction mixture was poured into dilute HCl (1 L) and extracted with ethyl acetate. The combined extracts were washed with water and dried. The reduced solution was chromatographed with 1:1 ethyl acetate:petrol on silica gel to give the product with a pale yellow solid, 11.7 g, 83%.

Preparation of N-(4-amino-3-hydroxyphenyl)-3,5-difluorosulphonylbenzenesulphonamide hydrochloride



N-[4-(3,5-bis-fluorosulphonylphenyl sulphamoyl)-2-hydroxyphenyl]acetanilide (4.7 g, 10.0 mmol) was added to a mixture of concentrated HCl (25 ml), water (40 ml) and tetrahydrofuran (40 ml). After heating under reflux for 6 hr, a clear (pale brown) solution was obtained. TLC (ethyl acetate) showed complete hydrolysis, and the product spot gave a positive amine test. The tetrahydrofuran was removed by evaporation to give a dark oily suspension that was redissolved with the aid of a little acetic acid. The material was used as such in the next stage.



The solution of N-(4-amino-3-hydroxyphenyl)-3,5-difluorosulphonylbenzenesulphonamide hydrochloride (nominally 10 mmol) was cooled to 10° C. or less in an ice bath, and a solution of sodium nitrite (0.76 g, 11.0 mmol) in water (5 ml) was added. After stirring for 10 min, a greyish solid formed, and urea was added to destroy excess nitrous acid. The cold mixture was then added dropwise to a cold, stirred solution of PC1 (four equivalent coupler COUP-1 with hydrogen at the coupling position: N-[4-chloro-3-[[4,5-dihydro-5-oxo-1-(2,4,6-trichlorophenyl)-1H-pyrazol-3-yl]amino]phenyl]-2-[3-(1,1-dimethylethyl)-4-hydroxyphenoxy]tetradecanamide) (8.56 g, 11.0 mmol) in tetrahydrofuran (150 ml) and pyridine (150 ml). By TLC, there was very little sign of any dye formation after 15 min, although the solution turned orange on continued stirring overnight. The reaction mixture was poured into dilute (10%) HCl (3 L) and extracted with ethyl acetate. The solvent was removed and replaced with THF (120 ml), and a solution of sodium hydroxide (4 g, 100 mmol) in water (20 ml) was added. After stirring for 20 min, the mixture was poured into dilute HCl (1 L), extracted with ethyl acetate, dried, and purified by chromatography on a silica gel pad. The solution was applied to the pad to absorb all the dye and then flushed with ethyl acetate until the washings were free of front running impurities. Then the pad was eluted with tetrahydrofuran to remove some of the product, followed with dimethyl formamide to remove the remaining product. The solvents were removed by rotary evaporation, and the residue dried by prolonged evacuation on a mechanical pump. The product coupler I-1 was obtained as a dark red-brown solid, total yield=9.82 g, 81%.

PHOTOGRAPHIC EXAMPLE 1

This example illustrates the photographic activity of masking coupler dispersion of a coupler I-1 in accordance with the invention relative to comparison coupler Comp1.

## 33

In each case the masking coupler (1.1 g) was first dissolved with slight heating in 56 ml of water containing 2% w/w 2-phenoxyethanol. The required amount of this solution was then mixed with gelatin and coating aids to constitute the melt containing coupler. A melt containing emulsion was prepared separately. The two melts were mixed in a dual mixer just prior to coating. The amounts of the various constituents were adjusted to give final laydowns of 344  $\mu\text{mol}/\text{m}^2$  (32  $\mu\text{mol}/\text{ft}^2$ ), 0.8  $\text{g}/\text{m}^2$  (75  $\text{mg}/\text{ft}^2$ ) and 2.7  $\text{g}/\text{m}^2$  (250  $\text{mg}/\text{ft}^2$ ) for coupler, silver and gelatin, respectively, on a film support. 35-mm strips from these coatings were exposed using a standard 21-step tablet and processed through the Kodak Flexicolor™ C-41 process, as described by *The British Journal of Photography Annual* of 1988, pp. 196-198, varying the time in the developer as indicated below. Another description of the use of the C-41 process is provided by *Using Kodak Flexicolor™ Chemicals*, Kodak Publication No. Z-131, Eastman Kodak Company, Rochester, N.Y. The processed film samples are subjected to Status M integral densitometry, and the Status M green and blue densities were then recorded. A second set of strips was processed without the bleach step to determine the amount of developed silver as a function of exposure. The following results were obtained.

| Coupler                                                  | I-1  |      |      | Comp1 |      |      |
|----------------------------------------------------------|------|------|------|-------|------|------|
| Time in Developer (s)                                    | 45   | 75   | 195  | 45    | 75   | 195  |
| Green Density Dmin (Min Exposure)                        | 0.17 | 0.20 | 0.38 | 0.20  | 0.39 | 1.06 |
| Green Density Dmax (Max Exposure)                        | 0.97 | 0.95 | 0.99 | 0.99  | 1.01 | 1.06 |
| Blue Density Dmin                                        | 0.69 | 0.66 | 0.58 | 0.64  | 0.52 | 0.26 |
| Blue Density Dmax                                        | 0.30 | 0.28 | 0.30 | 0.29  | 0.25 | 0.26 |
| Developed Silver in Dmin ( $\text{mg}/\text{m}^2$ )      | 14   | 28   | 32.2 | 16.1  | 59.2 | 273  |
| Hue of Masking Dye ( $\lambda_{\text{max}}, \text{nm}$ ) | 437  |      |      | 443   |      |      |

It is clear that the compound Comp1 which does not have a 2-hydroxyl substituent gives rise to a high level of silver fog (developed silver in Dmin) at high development times, resulting in a loss in discrimination between the low and high exposure regions of the strip (Dmin and Dmax). In contrast, the level of fog is significantly lower with the compound of this invention (I-1) and adequate discrimination is obtained. Furthermore, the compound I-1 also displays good activity and masking hue.



## PHOTOGRAPHIC EXAMPLE 2

A color negative film element 201 is prepared as follows. All coating coverages are reported in parenthesis in terms of

## 34

$\text{g}/\text{m}^2$ , except as otherwise indicated. Silver halide coating coverages are reported in terms of silver. The symbol "M %" indicates mol percent.

An aqueous solution of yellow colored magenta masking coupler I-1 of the invention is prepared as follows: Masking coupler I-1 (1.0 g) is dissolved in 8.4 ml of a solution containing 2% w/w 2-phenoxyethanol by gentle heating, resulting in a concentration of 10.7% by weight of I-1. A liquid coating solution is prepared by combining this solution with 181 g of distilled water. A final concentration of 0.53% I-1 by weight results. The solution is combined with other ingredients during extrusion coating to produce Sample 201 as described below.

## Sample 201

This sample is prepared by applying the following layers in the sequence recited to a transparent film support of cellulose triacetate with conventional subbing layers, with the red recording layer unit coated nearest the support. The side of the support to be coated is prepared by the application of gelatin subbing.

## Layer 1: AHU

|    |                                                |         |
|----|------------------------------------------------|---------|
| 25 | Black colloidal silver sol                     | (0.107) |
|    | UV-1                                           | (0.075) |
|    | UV-2                                           | (0.075) |
|    | Oxidized developer scavenger S-1               | (0.161) |
| 30 | Compensatory printing density cyan dye CD-1    | (0.034) |
|    | Compensatory printing density magenta dye MD-1 | (0.013) |
|    | Compensatory printing density yellow dye MM-1  | (0.095) |
|    | HBS-1                                          | (0.105) |
|    | HBS-2                                          | (0.399) |
|    | HBS-4                                          | (0.013) |
|    | Disodium salt of 3,5-disulfocatechol           | (0.215) |
|    | Gelatin                                        | (2.152) |

## Layer 2: SRU

This layer is comprised of a blend of a lower and higher (lower and higher grain ECD) sensitivity, red-sensitized tabular silver iodobromide emulsions respectively containing 1.5 M % and 4.1 M % iodide, based on silver.

|    |                                                      |         |
|----|------------------------------------------------------|---------|
| 45 | AgIBr (0.55 $\mu\text{m}$ ECD, 0.08 $\mu\text{m}$ t) | (0.355) |
|    | AgIBr (0.66 $\mu\text{m}$ ECD, 0.12 $\mu\text{m}$ t) | (0.328) |
|    | Bleach accelerator coupler B-1                       | (0.075) |
|    | DIR-1                                                | (0.015) |
| 50 | Cyan dye forming coupler C1                          | (0.359) |
|    | HBS-2                                                | (0.359) |
|    | HBS-3                                                | (0.030) |
|    | HBS-5                                                | (0.098) |
|    | TAI                                                  | (0.011) |
|    | Gelatin                                              | (1.668) |

## Layer 3: MRU

This layer is comprised of a red-sensitized tabular silver iodobromide emulsion containing 4.1 M % iodide, based on silver.

|    |                                                      |         |
|----|------------------------------------------------------|---------|
| 60 | AgIBr (1.30 $\mu\text{m}$ ECD, 0.12 $\mu\text{m}$ t) | (1.162) |
|    | Bleach accelerator coupler B-1                       | (0.005) |
|    | DIR-1                                                | (0.016) |
|    | Cyan dye forming magenta colored coupler CM-1        | (0.059) |
|    | Cyan dye forming coupler C1                          | (0.207) |
|    | HBS-2                                                | (0.207) |
|    | HBS-3                                                | (0.032) |
|    | HBS-5                                                | (0.007) |

-continued

|         |         |
|---------|---------|
| TAI     | (0.019) |
| Gelatin | (1.291) |

## Layer 4: FRU

This layer is comprised of a red-sensitized tabular silver iodobromide emulsion containing 3.7 M % iodide, based on silver.

|                                                      |         |
|------------------------------------------------------|---------|
| AgIBr (2.61 $\mu\text{m}$ ECD, 0.12 $\mu\text{m}$ t) | (1.060) |
| Bleach accelerator coupler B-1                       | (0.005) |
| DIR-2                                                | (0.048) |
| DIR-1                                                | (0.027) |
| Cyan dye forming magenta colored coupler CM-1        | (0.022) |
| Cyan dye forming coupler C1                          | (0.312) |
| HBS-1                                                | (0.194) |
| HBS-2                                                | (0.274) |
| HBS-3                                                | (0.054) |
| HBS-5                                                | (0.007) |
| TAI                                                  | (0.010) |
| Gelatin                                              | (1.291) |

## Layer 5: Interlayer

|                                  |         |
|----------------------------------|---------|
| Oxidized developer scavenger S-1 | (0.086) |
| HBS-4                            | (0.129) |
| Gelatin                          | (0.538) |

## Layer 6: SGU

This layer is comprised of a blend of a lower and higher (lower and higher grain ECD) sensitivity, green-sensitized tabular silver iodobromide emulsions respectively containing 2.6 M % and 4.1 M % iodide, based on silver.

|                                                      |         |
|------------------------------------------------------|---------|
| AgIBr (0.81 $\mu\text{m}$ ECD, 0.12 $\mu\text{m}$ t) | (0.251) |
| AgIBr (0.92 $\mu\text{m}$ ECD, 0.12 $\mu\text{m}$ t) | (0.110) |
| Magenta dye forming yellow colored coupler I-1       | (0.070) |
| Magenta dye forming coupler M1                       | (0.339) |
| Stabilizer ST-1                                      | (0.034) |
| HBS-1                                                | (0.305) |
| TAI                                                  | (0.006) |
| Gelatin                                              | (1.721) |

## Layer 7: MGU

This layer is comprised of a blend of a lower and higher (lower and higher grain ECD) sensitivity, green-sensitized tabular silver iodobromide emulsions each containing 4.1 M % iodide, based on silver.

|                                                      |         |
|------------------------------------------------------|---------|
| AgIBr (0.92 $\mu\text{m}$ ECD, 0.12 $\mu\text{m}$ t) | (0.113) |
| AgIBr (1.22 $\mu\text{m}$ ECD, 0.11 $\mu\text{m}$ t) | (1.334) |
| DIR-3                                                | (0.032) |
| Magenta dye forming yellow colored coupler I-1       | (0.154) |
| Magenta dye forming coupler M1                       | (0.087) |
| Oxidized developer scavenger S-2                     | (0.018) |
| HBS-1                                                | (0.079) |
| HBS-2                                                | (0.032) |
| Stabilizer ST-1                                      | (0.009) |
| TAI                                                  | (0.023) |
| Gelatin                                              | (1.668) |

## Layer 8: FGU

This layer is comprised of a green-sensitized tabular silver iodobromide emulsion containing 4.1 M % iodide, based on silver.

|    |                                                      |         |
|----|------------------------------------------------------|---------|
| 5  | AgIBr (2.49 $\mu\text{m}$ ECD, 0.14 $\mu\text{m}$ t) | (0.909) |
| 10 | DIR-4                                                | (0.003) |
|    | DIR-5                                                | (0.032) |
|    | Magenta dye forming yellow colored coupler I-1       | (0.070) |
|    | Magenta dye forming coupler M1                       | (0.113) |
|    | HBS-1                                                | (0.108) |
|    | HBS-2                                                | (0.065) |
|    | Stabilizer ST-1                                      | (0.011) |
|    | TAI                                                  | (0.011) |
|    | Gelatin                                              | (1.405) |

## Layer 9: Yellow Filter Layer

|    |                                  |         |
|----|----------------------------------|---------|
| 20 | Yellow filter dye YD-1           | (0.054) |
|    | Oxidized developer scavenger S-1 | (0.086) |
|    | HBS-4                            | (0.129) |
|    | Gelatin                          | (0.646) |

## Layer 10: SBU

This layer is comprised of a blend of a lower, medium and higher (lower, medium and higher grain ECD) sensitivity, blue-sensitized tabular silver iodobromide emulsions respectively containing 1.5 M %, 1.5 M % and 4.1 M % iodide, based on silver.

|    |                                                      |         |
|----|------------------------------------------------------|---------|
| 35 | AgIBr (0.55 $\mu\text{m}$ ECD, 0.08 $\mu\text{m}$ t) | (0.156) |
|    | AgIBr (0.77 $\mu\text{m}$ ECD, 0.14 $\mu\text{m}$ t) | (0.269) |
|    | AgIBr (1.25 $\mu\text{m}$ ECD, 0.14 $\mu\text{m}$ t) | (0.430) |
|    | DIR-1                                                | (0.027) |
|    | DIR-6                                                | (0.054) |
|    | Yellow dye forming coupler Y1                        | (1.022) |
|    | Bleach accelerator coupler B-1                       | (0.011) |
|    | HBS-1                                                | (0.538) |
|    | HBS-3                                                | (0.054) |
|    | HBS-5                                                | (0.014) |
|    | TAI                                                  | (0.014) |
|    | Gelatin                                              | (2.119) |

## Layer 11: FBU

This layer is comprised of a blue-sensitized silver iodobromide emulsion containing 9.0 M % iodide, based on silver.

|    |                                               |         |
|----|-----------------------------------------------|---------|
| 50 | AgIBr (1.04 $\mu\text{m}$ ECD)                | (0.699) |
|    | Unsensitized silver bromide Lippmann emulsion | (0.054) |
|    | Yellow dye forming coupler Y1                 | (0.473) |
|    | DIR-6                                         | (0.086) |
|    | Bleach accelerator coupler B-1                | (0.005) |
|    | HBS-1                                         | (0.280) |
|    | HBS-5                                         | (0.004) |
|    | TAI                                           | (0.012) |
|    | Gelatin                                       | (1.183) |

## Layer 12: Ultraviolet Filter Layer

|    |                                               |         |
|----|-----------------------------------------------|---------|
| 60 | Dye UV-1                                      | (0.108) |
|    | Dye UV-2                                      | (0.108) |
|    | Unsensitized silver bromide Lippmann emulsion | (0.215) |

-continued

|         |         |
|---------|---------|
| HBS-1   | (0.151) |
| Gelatin | (0.699) |

5

-continued

|                                            |         |
|--------------------------------------------|---------|
| Soluble polymethylmethacrylate maffe beads | (0.108) |
| Silicone lubricant                         | (0.039) |
| Gelatin                                    | (0.882) |

### Layer 13: Protective Overcoat Layer

This film is hardened at the time of coating with 1.80% by weight of total gelatin of hardener H-1. Surfactants, coating aids, soluble absorber dyes, antifoggants, stabilizers, anti-static agents, biostats, biocides, and other addenda chemicals are added to the various layers of this sample, as is commonly practiced in the art.

Polymethylmethacrylate maffe beads (0.005)

1

## Glossary of Acronyms

|       |                                                         |
|-------|---------------------------------------------------------|
| HBS-1 | Tritoluoyl phosphate                                    |
| HBS-2 | Di-n-butyl phthalate                                    |
| HBS-3 | N-n-Butyl avetanilide                                   |
| HBS-4 | Tris(2-ethylhexyl) phosphate                            |
| HBS-5 | N,N-Diethyl lauramide                                   |
| H-1   | Bis(vinylsulfonyl) methane                              |
| TAI   | 4-Hydroxy-6-methyl-1,3,3a,7-tetraazaindene, sodium salt |



-continued

## Glossary of Acronyms

Y1



DIR-1



DIR-2



DIR-3



-continued

## Glossary of Acronyms

DIR-4



DIR-5



DIR-6



CM-1



-continued

## Glossary of Acronyms

MM-1



MD-1



CD-1



-continued

## Glossary of Acronyms

B-1



YD-1



UV-1



UV-2



S-1



S-2



55

The invention has been described in detail with particular reference to preferred embodiments thereof, but it will be understood that variations and modifications can be effected within the spirit and scope of the invention.

60

We claim:

1. A multilayer silver halide color photographic element comprising a support bearing a light-sensitive silver halide emulsion layer and a non-diffusible yellow-colored magenta dye-forming masking coupler of the following formula

65

wherein



COUP is a magenta dye-forming coupler having the azo group attached to its coupling position; q is an integer of from 0 to 3, and each R' independently represents a substituent group or two R' groups together complete a ring of from 5-7 atoms; m is 1 or 2, and DG represents a substituent of the formula



where

each L<sup>1</sup> represents a divalent linking group; each k is either 0 or 1; each L<sup>2</sup> represents —NHSO<sub>2</sub>—, —NHCO—, —SO<sub>2</sub>NH—, or —CONH—; each Z represents —SO<sub>3</sub>M or —PO<sub>3</sub>M, where M represents H or a counter ion; and each n represents an integer of from 1 to 5;

with the provisos that each DG substituent group, when present, is located in the 4- or 6-position meta to the 2-hydroxyl substituent on the arylazo group, and that when at least one L<sup>1</sup> or L<sup>2</sup> group comprises an —NHSO<sub>2</sub>— or —SO<sub>2</sub>NH— group then the total number of Z group substituents on the coupler is at least 2, and when no L<sup>1</sup> or L<sup>2</sup> group comprises an —NHSO<sub>2</sub>— or —SO<sub>2</sub>NH— group then the total number of Z group substituents on the coupler is at least 3, and if k is 0 for a DG substituent group then the L<sup>2</sup> group for that DG substituent is either —NHSO<sub>2</sub>— or —NHCO—.

2. An element according to claim 1, wherein q is 0.

3. An element according to claim 1, wherein for at least one DG substituent, k is 1 and L<sup>1</sup> represents —O(CH<sub>2</sub>)<sub>y</sub>—, —NHCO(CH<sub>2</sub>)<sub>y</sub>—, or —NRCO(CH<sub>2</sub>)<sub>y</sub>—, where R represents an alkyl or aryl group and y represents an integer from 1 to 4.

4. An element according to claim 1, wherein k is 0.

5. An element according to claim 1, wherein for at least one DG substituent L<sup>2</sup> represents —NHSO<sub>2</sub>—.

6. An element according to claim 1, wherein each Z represents —SO<sub>3</sub>M.

7. An element according to claim 1, wherein the masking coupler is of the formula:



8. An element according to claim 1, wherein COUP is a 5-pyrazolone dye-forming coupler.

9. An element according to claim 1, wherein COUP is a 5-pyrazolone coupler having an anilino group in the 3-position.

10. An element according to claim 1, wherein COUP is represented by the structure:

(M-6)



where:

Ar is selected from the group consisting of unsubstituted aryl groups, substituted aryl groups and substituted pyridyl groups, the substituents being selected from the group consisting of halogen atoms and cyano, alkylsulfonyl, arylsulfonyl, sulfamoyl, sulfonamido, carbamoyl, carbonamido, alkoxy, aryloxy, aryloxy, alkoxy carbonyl, aryloxy carbonyl, ureido, nitro, alkyl, and trifluoromethyl groups, or Ar is an aryl or pyridyl group substituted with a group which forms a link to a polymeric chain;

Y is an anilino group substituted with one or more substituents selected from the group consisting of halogen atoms, and alkyl, aryl, alkoxy, aryloxy, carbonamido, carbamoyl, sulfonamido, sulfamoyl, alkylsulfinyl, arylsulfinyl, alkylsulfonyl, arylsulfonyl, alkoxy carbonyl, aryloxy carbonyl, acyl, acyloxy, ureido, imido, carbamate, heterocyclic, cyano, trifluoromethyl, alkylthio, nitro, carboxyl and hydroxyl groups, and groups which form a link to a polymeric chain, and wherein Y contains at least 6 carbon atoms; and

X represents the coupling-off position.

11. An element according to claim 1, wherein COUP comprises a ballast group of such size and configuration that, in combination with the remainder of the molecule, it provides the coupler with sufficient bulk to be substantially non-diffusible from the layer in which it is coated in the element.

12. An element according to claim 1, wherein the masking coupler is present in the element at a coverage of less than 0.4 mmol/m<sup>2</sup>.

13. An element according to claim 1, wherein the masking coupler is present in the element at a coverage of from 0.1 mmol/m<sup>2</sup> to 0.3 mmol/m<sup>2</sup>.

14. An element according to claim 1, wherein the colored coupler is of the formula:



15. An element according to claim 14, wherein q is 0.

16. An element according to claim 14, wherein q is an integer of from 1 to 3, and each R' independently represents a substituent group with a Hammett sigma-para value of less than 0.05, or two R' groups together complete a ring of from 5-7 atoms.

17. An element according to claim 14, wherein q is an integer of at least one and each R' group represents OR, R, NHCOR, 6—OH, 6—NHSO<sub>2</sub>R, or 6—NR<sub>2</sub>, where R represents an alkyl or aryl group.

**49**

**18.** An element according to claim **14**, wherein k is 1 and L<sup>1</sup> represents —O(CH<sub>2</sub>)<sub>y</sub>—, —NHCO(CH<sub>2</sub>)<sub>y</sub>—, or —NRCO(CH<sub>2</sub>)<sub>y</sub>—, where R represents an alkyl or aryl group and y represents an integer from 1 to 4.

**19.** An element according to claim **14**, wherein k is 0. <sup>5</sup>

**20.** An element according to claim **14**, wherein L<sup>2</sup> represents —NHSO<sub>2</sub>—.

**21.** An element according to claim **14**, wherein each Z represents —SO<sub>3</sub>M.

**22.** An element according to claim **14**, wherein COUP is a 5-pyrazolone dye-forming coupler. <sup>10</sup>

**23.** An element according to claim **14**, wherein COUP is a 5-pyrazolone coupler having an anilino group in the 3-position.

**24.** An element according to claim **14**, wherein COUP is represented by the structure: <sup>15</sup>

(M-6)



where:

Ar is selected from the group consisting of unsubstituted aryl groups, substituted aryl groups and substituted pyridyl groups, the substituents being selected from the group consisting of halogen atoms and cyano, alkylsulfonyl, arylsulfonyl, sulfamoyl, sulfonamido,

**50**

carbamoyl, carbonamido, alkoxy, acyloxy, aryloxy, alkoxy carbonyl, aryloxycarbonyl, ureido, nitro, alkyl, and trifluoromethyl groups, or Ar is an aryl or pyridyl group substituted with a group which forms a link to a polymeric chain;

Y is an anilino group substituted with one or more substituents selected from the group consisting of halogen atoms, and alkyl, aryl, alkoxy, aryloxy, carbonamido, carbamoyl, sulfonamido, sulfamoyl, alkylsulfonyl, arylsulfonyl, alkylsulfonyl, arylsulfonyl, alkoxy carbonyl, aryloxycarbonyl, acyl, acyloxy, ureido, imido, carbamate, heterocyclic, cyano, trifluoromethyl, alkylthio, nitro, carboxyl and hydroxyl groups, and groups which form a link to a polymeric chain, and wherein Y contains at least 6 carbon atoms; and

X represents the coupling-off position.

**25.** An element according to claim **14**, wherein COUP comprises a ballast group of such size and configuration that, in combination with the remainder of the molecule, it provides the coupler with sufficient bulk to be substantially non-diffusible from the layer in which it is coated in the element. <sup>20</sup>

**26.** An element according to claim **14**, wherein the masking coupler is present in the element at a coverage of less than 0.4 mmol/m<sup>2</sup>. <sup>25</sup>

**27.** An element according to claim **14**, wherein the masking coupler is present in the element at a coverage of from 0.1 mmol/m<sup>2</sup> to 0.3 mmol/m<sup>2</sup>. <sup>30</sup>

\* \* \* \* \*